

Aug. 15, 1944.

W. T. ENNOR

2,355,963

WIRE FABRIC

Original Filed July 16, 1940

Fig. 1.



Fig. 2.



INVENTOR

WILLIAM T. ENNOR

BY

*Edward B. Foste*  
ATTORNEY

## UNITED STATES PATENT OFFICE

2,355,963

## WIRE FABRIC

William Trehane Ennor, Newark, Ohio, assignor  
to Aluminum Company of America, Pittsburgh,  
Pa., a corporation of Pennsylvania

Continuation of application Serial No. 345,818,  
July 16, 1940. This application May 16, 1944,  
Serial No. 535,821

12 Claims. (Cl. 148—11.5)

This invention relates to wire fabric, and particularly to wire fabric made from wires of aluminum base alloys. By aluminum base alloys is meant those alloys containing at least 50 per cent aluminum. This application is a continuation of application Serial No. 345,818, filed July 16, 1940.

Because of aluminum's light weight, durability, attractive appearance, and non-staining characteristics, attempts have been made to make wire fabric from it and its alloys for use as screen cloth and the like. However, difficulty has been encountered in producing aluminum wire fabric which is suitable for commercial purposes. One of the principal difficulties has been that the fabric was "sleazy" and not stiff enough. The term "sleazy" refers to susceptibility of the fabric to be manipulated easily into a condition where the wires do not cross at right angles. Another problem has been to produce fabric which was sufficiently resistant to corrosion.

When, in order to obtain increased corrosion resistance and other desired properties, aluminum wire fabric is made from duplex wires consisting of a core of an aluminum base alloy enclosed in a coating of a softer alloy of a higher electrode potential than the core, the fabric is ordinarily extremely stiff, in contrast to the sleazy condition mentioned above. The fabric also frequently possesses a ridged or uneven appearance, and the weft wires may be unevenly spaced as a result of what is generally known in the wire fabric industry as "flyback."

It is an object of this invention to provide an improved aluminum wire fabric. It is a further object of this invention to provide an improved aluminum wire fabric made from duplex wires of the type mentioned above, which is neither too stiff nor too sleazy, and which is free from bulges and ridges and uneven spacing of the weft wires resulting from "flyback." It is a further object of this invention to provide aluminum wire fabric woven from duplex wires having an aluminum base alloy core and an aluminum base alloy coating around the core, the coating alloy of certain of the wires of the fabric having mechanical properties differing from those of the coating of the other wires in the fabric.

Referring to the accompanying drawing,

Fig. 1 is an elevation of wire fabric embodying my invention; and

Fig. 2 is an enlarged cross-section taken on the line II—II of Fig. 1.

My invention is predicated upon the discovery that when aluminum wire fabric is made from

duplex wire having a core of an aluminum base alloy and a coating thereon of another aluminum base alloy, the stiffness of the fabric can be controlled, and ridges or bulges in the fabric, as well as uneven spacing of the weft wires resulting from "flyback," can be avoided, by using a combination of warp and weft wires in which the coating metal of the warp wires differs in hardness from the coating metal of the weft wires. Thus, when aluminum wire fabric is made from such duplex wire, and the coating of the warp wires is harder than the coating of the weft or filler wires, the degree of stiffness of the cloth is less than it would be if the coating metal on both sets of wires were of equal hardness, and furthermore, any tendency toward uneven spacing of the weft wires and toward the formation of ridges or bulges in the cloth during the weaving of it is minimized.

It is preferred to make the warp and weft wires from duplex wire having a core of a suitable aluminum base alloy and a coating of another aluminum base alloy, the latter alloy being susceptible to having its mechanical properties changed by proper treatment. The wire which is to form the warp wires of the fabric, or that which is to form the weft wires, or both, can then be subjected to suitable treatments for producing warp and weft wires in which the surface of the warp wires is harder than the surface of the weft wires.

Many aluminum base alloys are susceptible to improvement in tensile strength, yield strength, and hardness by certain thermal treatments which cause soluble alloying elements to enter into solution in the aluminum base metal. Those elements can be retained in solution by a rapid or controlled cooling from the elevated temperature of the thermal treatment to room temperature, even though their solubility in the aluminum is actually lower at room temperature than the amount retained in solution after the cooling step. The elevated temperature treatment is known to those skilled in the art as a "solution heat treatment," and the alloys whose mechanical properties can be substantially improved by such thermal treatments are referred to as "heat treatable alloys." Generally speaking, the preferred solution heat treatment temperature varies with the condition and character of the alloy, but a range of between 400° C. and 550° C. includes practically all of the commercial solution heat treatments for aluminum base alloys.

In the preferred form of my invention the wire

fabric is made from aluminum wire consisting of a core of a strong aluminum base alloy which is not susceptible to having its mechanical properties substantially improved by a solution heat treatment (which alloys are hereinafter referred to as "non-heat treatable alloys"), the core having a coating thereon of a heat treatable aluminum base alloy.

Before the fabric is woven, that portion of the wire which is to form the warp wires of the fabric is subjected to a solution heat treatment, and that portion of the wire which is to form the weft wires is annealed, thereby softening the coating alloy on it. The wires normally are subjected to a final drawing operation to draw them to final size subsequent to the thermal treatments mentioned, and although the drawing operation results in substantial changes in the mechanical properties of the wire because of the working of the metal, the wires still show marked differences in surface hardness resulting from the thermal treatments described previously. A reduction of from 75 to 96 per cent in the cross-sectional area of the wire is desirable during this drawing operation. Following the final drawing operation on the warp wire it is preferred to subject it to an artificial aging treatment, which consists of heating the wire at a temperature between 100° C. and 200° C. This treatment increases the hardness of the coating alloy, and in addition, when the alloy forming the core contains magnesium, the ductility and percentage of elongation of the wire is increased, with the result that breakage of the wire during weaving is minimized. Ordinarily a treatment for about four hours at 118° C. is satisfactory for this step. The artificial aging treatment may precede the final drawing operation on the warp wire, but preferably follows the drawing operation.

The duplex wire giving the best results is that consisting of a core of an aluminum base alloy containing from 3-6 per cent magnesium, from 0.05-1 per cent manganese, and from 0.05-0.5 per cent chromium, the balance being aluminum plus impurities, which core has a coating of an aluminum base alloy containing from 0.5-3 per cent zinc, from 0.75-3 per cent magnesium silicide, and either from 0.05-.5 per cent chromium or from 0.1-1 per cent manganese, the balance being aluminum plus incidental impurities. With wire of the above described composition the hardness of the coating can be increased by a solution heat treatment, while the mechanical properties of the core are not substantially increased by the solution heat treatment. Prior to weaving the fabric, the wire which is to form the warp wires is subjected to a solution heat treatment by heating it at a temperature of about 510° C., as described in U. S. Patent 1,472-739 to Archer et al. The wire which is to form the weft wires is annealed by heating it at a temperature of about 250° C. to 400° C. in the manner well known in the art. Subsequent to the thermal treatments mentioned, I prefer to subject both sets of wire to a final drawing operation to draw the wire to the final size desired for the wire in the fabric. Following the final drawing operation the warp wire is preferably subjected to an artificial aging treatment, as described in the above-mentioned patent to Archer et al., with the result that the hardness of the coating, and the ductility and percentage of elongation of the core, are increased.

The particular temperatures most suitable for

the thermal treatments described above, and the duration of the thermal treatments, varies, depending on such factors as the particular composition and size of the wire and the size of the body of wire being treated. For most purposes a solution heat treatment at a temperature of 510° C. is satisfactory, and an anneal at 350° C. is adequate for the annealing treatment. After the solution heat treatment, the warp wire may be quenched from the solution heat treatment temperature by immersing it in water or oil, or by passing a current of air over it, in the manner well known in the art. Fabric woven from wires prepared in the manner described above is free from ridges or bulges, and has a degree of stiffness satisfactory for commercial purposes. Furthermore, the solution heat treated wires have a relatively hard surface, and consequently do not tend to become scratched during the weaving of the fabric, with the result that the wire has a smooth appearance. No rolling or other treatment of the woven fabric is necessary to prepare it for commercial use, but if desired, the fabric may be painted with aluminum paint or other types of paint.

Though the above described procedure for obtaining a difference in surface hardness of the warp and weft wires is preferred, various other known methods for achieving the difference in hardness may be employed. For example, both the warp and weft wires can be annealed to the same extent, so that their properties are similar, and then be subjected to a final drawing operation in which the weft wire is drawn to a lesser amount than the warp wire. As a result the weft wire is work-hardened by the drawing operation to a less extent than the warp wire, and consequently the coating on the warp wire is harder than the coating on the weft wire. To produce warp and weft wires of like cross-sectional dimensions and of differing hardness in this manner, the wires must be drawn prior to annealing to suitably differing cross-sectional dimensions to compensate for the difference in reduction in the final draw. Another method which can be used to obtain a difference in the properties of the two sets of wire is to soften the weft wire by annealing it following the final drawing operation, but not annealing the warp wire, with the result that the warp wire remains in the work-hardened condition.

In the accompanying drawing of wire fabric embodying my invention, the fabric consists of the warp wires 1 and the weft wires 2. The warp and weft wires consist of a core 3, which is composed of an aluminum base alloy, and a coating 4 of a different aluminum base alloy which has a higher electrode potential than the core. The warp and weft wires have been treated as described above prior to weaving the fabric, with the result that the coating on the warp wires is substantially harder than the coating on the weft wires.

As a specific example of my invention, wire fabric was made of duplex wire composed of a core having a composition of 0.1 per cent manganese, 5.25 per cent magnesium, 0.1 per cent chromium, and the balance aluminum plus incidental impurities. The coating on the core consisted of an alloy having a composition of 0.25 per cent chromium, 2 per cent zinc, 1.9 per cent magnesium silicide, and the balance aluminum plus impurities. That portion of the wire which was to form the warp wires of the fabric was given a

solution heat treatment at a temperature of 510° C., and then quenched in hot water. It was next subjected to a final drawing operation which reduced the wire from a diameter of .064 of an inch to .015 of an inch, and thereafter was heated for four hours at a temperature of 118° C. The wire which was to form the weft wires of the fabric was annealed by heating it at a temperature of 350° C. After it had cooled, it was subjected to a final drawing operation similar to that which was given the warp wire, reducing the diameter of the wire from .064 of an inch to .015 of an inch. The two sets of wire were then woven into wire fabric, and that fabric was flat and uniform in appearance, and was neither too stiff nor too "sleazy" for commercial use.

If a combination of duplex wires is used in which the surface of the weft wire is harder than the surface of the warp wire, the stiffness of the fabric is greater than is the case when the warp and weft wires are of equal hardness. Although ordinarily the problem with fabric made of duplex aluminum wires is to decrease the stiffness, it is sometimes advantageous to obtain an increase in stiffness, as where the fabric is made from wire of extremely small diameter or there is a large distance between the wires. In such case it is desirable to increase the stiffness of the fabric, and this may be accomplished by weaving the fabric from wire in which the surface of the weft wires is harder than the surface of the warp wires. The difference in surface hardness can, of course, be obtained by the methods described previously, but in this case the process for increasing the surface hardness of the duplex wire is applied to the weft wire and the process for softening the surface is used on the warp wire.

I claim:

1. Wire fabric comprising warp wires and weft wires, said wires comprising an aluminum base alloy core having a coating of a different aluminum base alloy, the coating on one set of wires being of different hardness than the underlying core, and the coating on the warp wires being of different hardness than the coating on the weft wires.

2. Wire fabric comprising warp wires and weft wires, said wires comprising an aluminum base alloy core having a coating of a different aluminum base alloy, the coating on the warp wires being of different hardness than the underlying core and harder than the coating on the weft wires.

3. Wire fabric comprising warp wires and weft wires, said wires comprising an aluminum base alloy core having a coating of a different aluminum base alloy, the coating on the warp wires being softer than the coating on the weft wires, and the coating on the weft wires having a different hardness than the underlying core.

4. Wire fabric comprising warp wires and weft wires, said wires comprising a core of a non-heat treatable aluminum base alloy having a coating of a heat treatable aluminum base alloy thereon, one of said sets of wires having a solution heat treated coating of different hardness than the underlying core, and the other set of wires being in the softened condition resulting from annealing thereof.

5. Wire fabric comprising warp wires and weft wires, said wires comprising a core composed of an aluminum base alloy having a coating thereon of a heat treatable aluminum base alloy, one of

said sets of wires having a solution heat treated coating, and the coating on the other set of wires being in the softened condition resulting from annealing thereof, the core of the wire having the solution heat treated coating being of different hardness than the solution heat treated coating.

6. Wire fabric comprising warp wires and weft wires, said wires comprising a core of a non-heat treatable aluminum base alloy having a coating of a heat treatable aluminum base alloy thereon, the coating of one of said sets of wires being in the solution heat treated and subsequently drawn condition, and the coating of the other set of wires being in the condition resulting from the wire being annealed to soften it and then wire-drawn, said first mentioned coating being harder in the drawn condition than said second mentioned coating.

7. Wire fabric comprising warp and weft wires, said wires comprising a core composed of an aluminum base alloy having a coating thereon of a heat treatable aluminum base alloy, the coating of one of said sets of wire being in the solution heat treated and subsequently drawn condition, and the coating of the other set of wires being in the condition resulting from the wire being annealed to soften it and then wire-drawn, said first mentioned coating being of different hardness than the underlying core and harder than said second mentioned coating.

8. In the method of making aluminum wire fabric in which the warp wires and weft wires comprise an aluminum base alloy core having a coating of a heat treatable aluminum base alloy, the steps comprising subjecting the wire for one of said sets of wires to a solution heat treatment and subsequently subjecting it to a wire-drawing operation, the coating alloy of the resultant material being of different hardness than the core, subjecting the wire for the other of said sets of wire to an annealing treatment, whereby the coating alloy thereof is softened, and subsequently subjecting it to a wire-drawing operation, whereby the coating of one of said sets of wires differs in hardness from the coating of the other set, and thereafter weaving wire fabric from the wires.

9. In the method of making aluminum wire fabric in which the warp wires and weft wires comprise an aluminum base alloy core having a coating of a heat treatable aluminum base alloy, the steps comprising subjecting wire which is to form warp wires of the fabric to a solution heat treatment and subsequently subjecting it to a wire-drawing operation, the coating alloy of the resultant material being of different hardness than the core, subjecting the wire which is to form weft wires of the fabric to an annealing treatment, whereby the coating alloy thereof is softened, and subsequently subjecting it to a wire-drawing operation, whereby the coating of one set of wires differs in hardness from the coating of the other set, and thereafter weaving wire fabric from the wires.

10. In the method of making aluminum wire fabric in which the warp wires and weft wires comprise an aluminum base alloy core having a coating of a heat treatable aluminum base alloy, the steps comprising subjecting the wire for one of said sets of wire to a solution heat treatment, thereafter subjecting it to a wire-drawing operation, and subsequently heating it at a temperature of from 100 to 200° C., the coating alloy of the resultant material being of different hardness

than the core, subjecting the wire for the other of said sets of wire to an annealing treatment, whereby the coating alloy thereof is softened, and subsequently subjecting it to a wire-drawing operation, whereby the coating of one of said sets of wires differs in hardness from the coating of the other set, and thereafter weaving wire fabric from the wires.

11. In the method of making aluminum wire fabric in which the warp wires and weft wires comprise an aluminum base alloy core having a coating of a heat treatable aluminum base alloy, the steps comprising subjecting the wire which is to form the warp wires to a solution heat treatment, thereafter subjecting it to a wire-drawing operation, and subsequently heating it at a temperature of from 100 to 200° C., the coating alloy of the resultant material being of different hardness than the core, subjecting the wire which is to form the weft wires to an annealing treatment, whereby the coating alloy thereof is softened, and subsequently subjecting it to a wire-drawing operation, whereby the coating of the

warp wire is harder than the coating of the weft wire, and thereafter weaving wire fabric from the wires.

12. In the method of making aluminum wire fabric in which the warp wires and weft wires comprise a non-heat treatable aluminum base alloy core having a coating of a heat treatable aluminum base alloy, the steps comprising subjecting the wire for one of said sets of wire to a solution heat treatment, subsequently subjecting it to a wire-drawing operation, and thereafter heating it at a temperature of from 100 to 200° C., the coating alloy of the resultant material being of different hardness than the core, subjecting the wire for the other of said sets of wire to an annealing treatment, whereby the coating alloy thereof is softened, and subsequently subjecting it to a wire-drawing operation, whereby the coating of one of said sets of wire differs in hardness from the coating of the other set, and thereafter weaving wire fabric from the wires.

WILLIAM TREHANE ENNOR.